

## UNITED STATES PATENT OFFICE

2,493,579

SOLUTION FOR ANODIC POLISHING OF  
STEEL AND IRON ARTICLES

Milton B. Hammond, Edgeworth, and Glade B. Bowman, Coraopolis, Pa., assignors to Standard Steel Spring Company, Coraopolis, Pa., a corporation of Pennsylvania

No Drawing. Application March 8, 1947,  
Serial No. 733,426

7 Claims. (Cl. 204—140.5)

1

This invention relates to a solution for use in the anodic electrolytic polishing of steel and iron articles. In such processes the steel or iron article is immersed in a solution and an electric current is passed from the article through the solution to a cathode. Various solutions have been employed in the anodic polishing of such articles but they are open to certain objections. Where a phosphoric acid solution is employed, it operates satisfactorily until a certain concentration of iron phosphate in solution has been reached but after that time the solution becomes green and a red deposit is formed on the steel article. We have found that by including sulphate ion in proper amount in a solution in which phosphoric acid is the principal constituent, we can cause the precipitation of iron sulphate from solution so as to maintain the concentration of iron in solution below a certain critical value such that the solution operates satisfactorily in polishing the steel. We have found that the iron metal in solution should be maintained below one ounce per gallon for satisfactory results.

In accordance with our invention, we include in a bath which consists principally of phosphoric acid, sodium sulphate or other alkali metal or ammonium sulphate in such amount as to react with the iron in solution and precipitate it and maintain the concentration of iron metal in solution below one ounce per gallon. It is preferred that the solution also contain a small amount of sulphuric acid, i. e., up to 4% by weight of the solution, but the sulphuric acid can be omitted provided there is sufficient alkali metal or ammonium sulphate present to maintain the iron in solution below the critical value.

A preferred solution according to our invention is as follows, all percentages being by weight and in the case of the acids, we mean per cent by weight of 100% acid. Of course the acid employed need not be of 100% strength but can be of the strength commercially available.

## Example

|                           | Per cent by weight |
|---------------------------|--------------------|
| Phosphoric acid.....      | 68                 |
| Sulphuric acid.....       | 4                  |
| Water .....               | 24                 |
| Tri-sodium phosphate..... | 2                  |
| Sodium sulphate.....      | 2                  |
| Gelatin .....             | 0.5                |

2

The solution may contain the ingredients within ranges as follows:

|                           | Range                                | Preferred Range     |
|---------------------------|--------------------------------------|---------------------|
| 5                         |                                      |                     |
| Phosphoric Acid.....      | Percent<br>55 to 85                  | Percent<br>60 to 70 |
| Sulphuric Acid.....       | 0.1 to 4                             | 1 to 4              |
| Water .....               | 7 to 30                              | 15 to 30            |
| Tri-sodium Phosphate..... | 1 to 15                              | 1 to 5              |
| 10                        | Sodium Sulphate.....<br>at least 0.5 |                     |

As mentioned previously, the sulphuric acid may be omitted entirely provided there is sufficient sodium sulphate or its equivalent to maintain the iron in solution below the critical value. The amount of sodium sulphate or its equivalent depends upon the amount of iron in solution. The solution will operate satisfactorily at the start of the process without any sodium sulphate or sulphuric acid, but after a time it is necessary to provide the sulphate ion required to cause precipitation of the iron thereby keeping the iron in solution below the critical value. In general, the sodium sulphate should amount to at least 0.5% and it is preferred that the sodium sulphate be present in such amount as to saturate the bath and leave an excess of undissolved sodium sulphate in the solution. This excess acts as a reservoir for supplying the sulphate ion required for maintaining the iron in solution below the critical value. There is no upper limit to the amount of sodium sulphate which the bath may contain since it is desirable to have an excess in solid form.

35 While sulphuric acid is not essential, provided there is sufficient sodium sulphate or its equivalent present, the preferred solution contains some sulphuric acid but not over 4%.

40 In place of sodium sulphate, we may employ other alkali metal or ammonium sulphates, for example, potassium sulphate, lithium sulphate and ammonium sulphate.

45 The tri-sodium phosphate reduces the chemical attack of the solution on the article before current is applied and increases the polishing action after current is applied. In general, the amount of tri-sodium phosphate should be increased as the percentage of water in the solution increases. In place of tri-sodium phosphate, we may use other tri-alkali phosphates, di-alkali

## 3

phosphate, mono-alkali phosphates or phosphorus pentoxide.

In order to aid in flocculating and causing the iron sulphate precipitate to settle, the solution preferably contains a small amount of gelatin or other suitable flocculating agent. The preferred bath contains about 0.5% of gelatin but amounts of flocculating agent within the range of 0.1% to 5% may be used.

In using the solution in the anodic polishing of steel, it is preferred to carry out the process at an anode current density of about 285 amps. per square foot and at a temperature of about 190° F. However, the solution may be used under widely varying conditions, the anode current density being as low as 25 or as high as 2000 amps. per square foot and the temperature can be any temperature up to about 250° F. The time for polishing the steel will vary depending upon the polish required, from about 1 minute to 20 minutes, the usual period being about 5 minutes.

The invention is not limited to the preferred ingredients or proportions but may be otherwise embodied or practiced within the scope of the following claims.

We claim:

1. A solution for use in the electrolytic polishing of steel and iron articles wherein the article is employed as an anode, said solution consisting essentially of and containing by weight 55 to 85% phosphoric acid, 7 to 30% water, 1 to 15% of a member of the class consisting of tri-alkali metal phosphate, di-alkali metal phosphate, mono-alkali metal phosphate, and phosphorus pentoxide, and at least 0.5% of a sulphate of the class consisting of alkali metal sulphate and ammonium sulphate.

2. A solution for use in the electrolytic polishing of steel and iron articles wherein the article is employed as an anode, said solution consisting essentially of and containing by weight 55 to 85% phosphoric acid, 0.1% to 4% sulphuric acid, 7 to 30% water, 1 to 15% of a member of the class consisting of tri-alkali metal phosphate, di-alkali metal phosphate, mono-alkali metal phosphate, and phosphorus pentoxide, and at least 0.5% of a sulphate of the class consisting of alkali metal sulphate and ammonium sulphate.

3. A solution for use in the electrolytic polishing of steel and iron articles wherein the article is employed as an anode, said solution consisting essentially of and containing by weight 55 to 85% phosphoric acid, 1% to 4% sulphuric acid, 7 to 30% water, 1 to 15% tri-sodium phosphate, and at least 0.5% of alkali metal sulphate.

4. A solution for use in the electrolytic polishing of steel and iron articles wherein the article is employed as an anode, said solution consisting

## 4

essentially of and containing by weight 55 to 85% phosphoric acid, 0.1% to 4% sulphuric acid, 7 to 30% water, 1 to 15% tri-sodium phosphate and at least 0.5% alkali metal sulphate.

5. A solution for use in the electrolytic polishing of steel and iron articles wherein the article is employed as an anode, said solution consisting essentially of and containing by weight 55 to 85% phosphoric acid, 7 to 30% water, 1 to 15% of a member of the class consisting of tri-alkali metal phosphate, di-alkali metal phosphate, mono-alkali metal phosphate, and phosphorus pentoxide, and a sulphate of the class consisting of alkali metal sulphate and ammonium sulphate, said sulphate being present in amount sufficient to at least saturate the solution.

6. A solution for use in the electrolytic polishing of steel and iron articles wherein the article is employed as an anode, said solution consisting essentially of and containing by weight 55 to 85% phosphoric acid, 0.1% to 4% sulphuric acid, 7 to 30% water, 1 to 15% tri-sodium phosphate and alkali-metal sulphate in amount sufficient to at least saturate the solution.

7. A solution for use in the electrolytic polishing of steel and iron articles wherein the article is employed as an anode, said solution consisting essentially of and containing by weight 55 to 85% phosphoric acid, 0.1% to 4% sulphuric acid, 7 to 30% water, 1 to 15% of a member of the class consisting of tri-alkali metal phosphate, di-alkali metal phosphate, mono-alkali metal phosphate and phosphorus pentoxide, 0.1% to 5% of a flocculating agent for iron sulphate, and at least 0.5% of a sulphate of the class consisting of alkali metal sulphate and ammonium sulphate.

MILTON B. HAMMOND.  
GLADE B. BOWMAN.

## REFERENCES CITED

The following references are of record in the file of this patent:

## UNITED STATES PATENTS

|    |           |        |                |
|----|-----------|--------|----------------|
| 45 | Number    | Name   | Date           |
|    | 2,330,170 | Manuel | Sept. 21, 1943 |

## FOREIGN PATENTS

|    |         |               |               |
|----|---------|---------------|---------------|
| 50 | Number  | Country       | Date          |
|    | 521,290 | Great Britain | May 17, 1940  |
|    | 547,592 | Great Britain | Sept. 2, 1942 |
|    | 556,797 | Great Britain | Oct. 21, 1943 |

## OTHER REFERENCES

55 "Iron Age," May 30, 1940, pages 26 through 30.  
"Proceedings of The American Electroplaters' Society," 1941, pages 109, 110.